

# UNITED STATES PATENT OFFICE.

EUGENE P. SCHOCH, OF AUSTIN, TEXAS.

## PROCESS OF OBTAINING ILLUMINATING-GAS FROM LIGNITE.

1,364,455.

Specification of Letters Patent.

Patented Jan. 4, 1921.

No Drawing.

Application filed August 30, 1919. Serial No. 320,930.

To all whom it may concern:

Be it known that I, EUGENE P. SCHOCH, a citizen of the United States, residing at Austin, in the county of Travis and State 5 of Texas, have invented certain new and useful Improvements in Processes of Obtaining Illuminating-Gas from Lignite; and I do hereby declare the following to be a full, clear, and exact description of the in- 10 vention, such as will enable others skilled in the art to which it appertains to make and use the same.

This invention relates to a process of obtaining an illuminating gas directly from lignite, without having to enrich the same, 15 and has for its object to improve the procedures heretofore proposed.

With this and other objects in view the invention consists in the novel steps and 20 combinations of steps constituting the process, all as will be more fully hereinafter disclosed and particularly pointed out in claims.

In order that the exact invention may be 25 the more clearly understood it is said: The gas ordinarily obtained through the dry distillation of lignite, such for example as that found in Texas, has a calorific power of say from 400 to 450 British thermal units (here- 30 inafter referred to as B. T. U.) per cubic foot, although some investigators put it as high as 450 B. T. U. This gas upon investigation may be shown to contain say from 18% to 22% of carbon dioxid,  $CO_2$ , and 35 therefore by removing the latter, the calorific power of said gas can be raised to say 500 to 550 B. T. U. But as is well known these figures are too small for a satisfactory illuminating gas, which latter requires a 40 calorific power of at least 600 B. T. U.

Therefore it has been heretofore proposed to suitably enrich the gases obtained from lignite when they are to be employed for illuminating purposes, but such procedure 45 is expensive and is attended by other objections not necessary to mention.

It has further been proposed to secure a rich gas by heating the lignite to various high temperatures in a retort, and by taking 50 off separately the various gases correspond- ing to the said temperatures, in the belief that some of the fractions thus obtained would be sufficiently rich in calories to be used as a city illuminating gas.

But I have found from practical tests

that as the lignite rises in temperature the only portion of the gas given off that is rich enough for a city gas, is evolved at a relatively low temperature and is relatively small in amount, or as low in volume as say 60 one fifteenth ( $\frac{1}{15}$ ) of the total. I have further found that those portions of the gas evolved from the lignite after this said rich portion, have heating powers of only about 430 B. T. U. that they amount in volume to 65 about 4500 cubic feet per ton of lignite, while those portions evolved before this said rich portion, have heating powers lower than 430 B. T. U. and amount to about 1000 cubic feet per ton.

It will thus be seen that out of say, 5900 70 cubic feet of gas per ton of lignite obtained by this method only a negligible fraction (about 400 cubic feet) is really rich enough to be used directly as a city gas and no 75 amount of fractionation can change the results.

Upon a further investigation of these 80 fractions, I have found that the percentage of hydrogen present, increases rather sud- denly, from about 15% to 30% or more, and that the carbon monoxid  $CO$  present also increases, both at approximately the same or slightly different temperatures as that at which the carbon dioxid  $CO_2$  decreases. 85 That is to say when employing what is known as Bastrop lignite and when the inside of the retort just above the lignite was at a temperature of 325° C. and the inside bottom of the retort was at a temperature 90 of 590° C., I found the percentage of car- bon dioxid  $CO_2$  present, to decrease sud- denly from say 40% to say 20% or less, also that the amounts of methane, ethane and 95 illuminants also decreased markedly, and that these decreases occurred at about the same temperature at which the hydrogen and carbon monoxid increased. I found substantially the same phenomena when using what is known as Milam Co. lignite 100 when the inside of the retort just above the lignite was at a temperature of 310° C. and the inside bottom of the retort was at a temperature of 575° C.

Upon still further examining these gas 105 fractions it became apparent that these changes in composition are so related, or are so balanced each against the other as to leave the heating power of the total volume of gas about the same or at say 430 B. T. U. 110

if we consider the Bastrop lignite. It further became apparent that the low heating powers of the gas portions evolved at high temperatures or after the  $\text{CO}_2$  has markedly decreased are not due to the presence of carbon dioxid while the low heating powers of said gas portions evolved at low temperatures are due to the presence of very high percentages of carbon dioxid. In other words these discoveries show that if the later fractions can be separated from the earlier, and the earlier separated from their  $\text{CO}_2$  content, then the earlier will have a high heating power.

15 In pursuing my tests I still further discovered that I could collect samples of gas at the lower temperatures which contained as much as 30%  $\text{CO}_2$  and which with this  $\text{CO}_2$  present had a heating power as high as 450 20 B. T. U.

In fact from average tests made on Milam Co. lignite I obtained an earlier gas fraction having 32%  $\text{CO}_2$  and a heating power of 455.5 B. T. U. when burned with its  $\text{CO}_2$  present. Having reached this result, it immediately followed that if I removed this content of  $\text{CO}_2$  from these earlier or lower temperature fractions I would obtain a large volume of gas having the desired high heating power above 600 B. T. U.

Accordingly in carrying out my invention I obtain a city illuminating gas having a heating power above 600 B. T. U. and in relatively large proportions directly from lignite by subjecting the latter to a destructive distillation in a retort, and separating out the lower temperature fractions or those fractions which are relatively rich in carbon dioxid from the higher temperature fractions; or those fractions which are relatively poor in carbon dioxid. The exact percentage of carbon dioxid which determines the dividing line between the lower and higher fractions, will depend upon the 45 particular richness desired in the city gas. If only a heating power of 600 B. T. U. is desired, then a simple calculation will show how low the last portions of the gas collected can be in  $\text{CO}_2$  in order that the average of that 50 collected will show 600 B. T. U. after all the  $\text{CO}_2$  has been removed. On the other hand if a higher heating power than 600 B. T. U. is desired or a heating power up to say 670 B. T. U. then that portion of the evolved gas 55 that will be selected for a city gas will show such a high percentage of  $\text{CO}_2$  as will, when removed, permit the gas to yield the desired heating power. For example the particular earlier fractions mentioned above as 60 containing 32%  $\text{CO}_2$  showed by both calculations and test that when the  $\text{CO}_2$  was removed it had a heating power of 670 B. T. U. A later fraction might have showed such a low percentage of  $\text{CO}_2$  that when burned 65 without said  $\text{CO}_2$  its heating power would

be below 600 B. T. U. yet if this said later fraction were separated with said earlier fraction the two could easily show a heating power after the removal of the  $\text{CO}_2$  well above 600 B. T. U.

70 It will now be clear that my process involves the recovery and separation of lower fractions of gas that are so rich in  $\text{CO}_2$  that when burned with their  $\text{CO}_2$  content they will yield calorific powers well below 600 75 B. T. U., but on the other hand when burned without their  $\text{CO}_2$  content they are so rich in constituents of high heat giving powers that they will yield a calorific power above 600 B. T. U.

80 The separation of the carbon dioxid from the recovered city gas making fractions may be accomplished in any suitable manner, as for example, by passing the gas through a potassium carbonate solution. I have found 85 no difficulty in thus reducing the amount of  $\text{CO}_2$  present down to say 1% and thus raising the heating power of the city fraction gas from say 450 B. T. U. to 647 B. T. U. After the potassium carbonate solution has 90 thus become saturated with carbon dioxid, it may be regenerated in the usual manner by heating it until the absorbed carbon is expelled; and then it may be used over again. The heat used for this regenerating purpose 95 is the main operating cost encountered but it may be obtained from the waste gases of the process that are too poor for other purposes.

I have further discovered that in carrying out this process for making a city gas from lignite, practically the whole of the tar that is formed in the retorting operation is obtained during the formation of this city gas making fraction, so said tar is recovered as a by product, and goes to partially defray the expense of the operation. That is to say, the economic retorting of lignite requires the preparation and disposition of all products, and among these are the "coke" residue, and the tar. The "coke" residue should be as rich in combustible components as possible, provided it is of such a nature that briquets made from it will not "explode" or disintegrate in a fire. Such a coke residue is obtained if the retorting is discontinued after removing the fraction I convert into a city gas. And, at the same time, I secure all of the tar, from which I may make various valuable 110 products such as oils, paraffin, or asphaltic residues for briquet binders, etc.

115 It is obvious that those skilled in the art may vary the foregoing procedure without departing from the spirit of the invention, therefore I do not wish to be limited to the above disclosure except as may be required by the claims.

120 What I claim is:

1. The process of making an illuminating 125

gas from lignite which consists in subjecting said lignite to a fractional distillation until the percentage of carbon dioxid evolved shows a marked decrease, thereby 5 evolving at lower temperatures producing fractions of gases of relatively high illuminating powers mixed with substantial percentages of carbon dioxid; recovering said fractions; and removing the carbon dioxid 10 present from said fractions, substantially as described.

2. The process of making an illuminating gas from lignite which consists in subjecting said lignite to a distillation process 15 until the percentage of carbon dioxid evolved with the other gases shows a marked decrease; collecting all the gases thus produced; and separating out the carbon dioxid present, substantially as de- 20 scribed.

3. The process of making an illuminating gas having a calorific power exceeding six hundred British thermal units, which consists in subjecting lignite to a distillation 25 process of increasing temperatures and until the percentage of carbon dioxid evolved with the other gases begins to rapidly decrease; collecting the gases thus produced; and separating out the carbon dioxid pres- 30 ent, substantially as described.

4. The process of making an illuminating gas having a calorific power exceeding six hundred British thermal units, which consists in subjecting lignite to a fractional dis-

tillation process of increasing temperatures 35 and until the percentage of carbon dioxid evolved with the other gases decreases by as much as five per cent.; collecting the gases thus produced; and separating out the carbon dioxid present, substantially as de- 40 scribed.

5. The process of making an illuminating gas having a calorific power exceeding six hundred British thermal units, which consists in subjecting lignite to a distillation 45 process of increasing temperatures and until the temperature of the lignite exceeds 290° and the percentage of carbon dioxid evolved with the other gases has substantially de- 50 creased; collecting the gases thus produced; and separating out the carbon dioxid present, substantially as described.

6. The process of making an illuminating gas suitable for city use directly from lignite which consists in subjecting said lignite to fractional distillation until the percentage of carbon dioxid evolved shows a marked decrease; separating out those fractions of the evolved gases which are rich in carbon dioxid; and removing said carbon 60 dioxid from the gases thus recovered, substantially as described.

In testimony whereof I affix my signature, in presence of two witnesses.

EUGENE P. SCHOCH.

Witnesses:

R. A. MCNEES,  
ROBERT S. TAYLOR.